

106/165  
Patented Mar. 28, 1944

2,345,211

## UNITED STATES PATENT OFFICE

2,345,211

## INVESTMENT COMPOSITION

Robert Neiman, Louisville, Ky., assignor to  
Edmund A. Steinbock, Louisville, Ky.No Drawing. Application July 16, 1941,  
Serial No. 402,699

10 Claims. (Cl. 22—188)

This invention relates to investment compositions for use in making refractory molds into which metals or alloys may be cast into objects of a predetermined size and shape.

The compositions given herein have general application in the casting of many metals, but will, however, be described in detail for use in casting metallic alloy dentures.

In making a cast metallic denture, the investment composition is first formed into a model resembling the mouth structure and includes either the upper or lower portion of the mouth. On this model the denture to be constructed is first formed in wax. This is properly sprued and then this model is encased in another mix of investment, thus forming the complete mold. An entrance or crucible chamber is formed so that the molten metal may enter the sprue hole or holes and thence form the casting itself. This mold is heated to such temperature as will melt and carbonize the wax, remove all moisture present, and thence generally to a temperature as will promote expansion of the mold and provide a mold hot enough to permit the entering molten metal to reach recesses of the cavity, formed by the removal of the wax, and before the said molten metal solidifies. The mold is thence placed in a suitable casting machine, the metal is melted, and then poured or cast under pressure. After the metal solidifies and the mold cools sufficiently it is broken apart and the casting recovered.

In order to carry out this procedure with the best results, it is necessary that the investment composition form a plastic mass that is readily formed into the desired shape. The investment should have the property of forming a very smooth and refractory surface in contact with the wax pattern so that the cast denture will be as smooth as possible and free from reaction products between the molten metal and refractory.

The investment should provide about 3 to 5 minutes working time while in the plastic state and then should harden sufficiently for safe use in 30 minutes to 1 hr. The strength of the investment at the end of this latter period should be such that it may be safely used without the necessity of drying or dipping in molten waxes. Upon setting, the surface should not become unduly powdery and should promote adherence of the wax as much as possible.

For casting dentures, it is most desirable to have high thermal expansion, that is, between 1 and 2%, between room temperature and casting temperature. While being heated, the mold should expand fairly regularly and at no time should shrink appreciably below its original size. At the same time, the mold should not crack during the heating period.

When making the original model upon which the denture is built (in wax), the investment

should not change appreciably in size upon setting. Its setting expansion should be preferably between 0.0% and 0.1%. While slight shrinkage and positive expansions up to 0.2% are not extremely harmful, they, nevertheless, tend to produce undesirable distortion in the models.

The principal ingredient of an investment is the refractory filler, since it is this material that provides the refractory properties necessary and promotes desirable expansion of the mold. For some purposes, it is desirable to have greater refractoriness without expansion. For other purposes, for example, in dentistry, it is necessary to provide high refractoriness with high thermal expansion.

One of the objects of this invention is to provide a composition of materials to meet all of the above mentioned exacting specifications.

Another object of this invention is to provide investments of practically zero setting expansion and with almost any desired thermal expansion.

Another object is to provide an improved binder for use with a wide variety of refractory fillers.

Still another object of this invention is to provide a bond that will be very strong at room temperature and yet will not become much stronger nor vitrified on heating so that it may be removed from the casting without injuring the latter.

As was mentioned above, the principal ingredient of an investment composition is the refractory filler, and the one most generally used, is silica. It is available in a number of forms including quartz, tridymite, cristobalite, and fused quartz. Some of the more impure forms containing amorphous materials include chalcedony, flint, chert, opal, jasper, and diatomaceous earth. Of these forms, cristobalite has the greatest thermal expansion, with tridymite and quartz having a somewhat lower expansion with the latter combining good expansion with low price and a wide variety of particle sizes.

Clays, especially of a refractory nature, and grog, are widely used in industry but are not so satisfactory for the molds described herein when used in large quantities due to their shrinkage or low expansion. They may be used where this disadvantage is not very material. Aluminum oxide in its various hydrated and, better yet, in the calcined and fused state, makes a good refractory. Other refractories that may be used

alone or in a wide variety of mixtures include iron ore, (chiefly hematite and magnetite), other refractory natural ores, olivine, forsterite, cordierite, pyroxenes, spinels, berillium oxide, cerium oxide, lanthanum oxide, thorium oxide, yttrium oxide, zircon. Many of the carbides are sometimes useful and include those of silicon, molybdenum, hafnium, tantalum, titanium, tungsten, and zirconium. The nitrides and borides of the aforementioned metals also are quite refractory. Car-

bon (especially as graphite) and chromite, are valuable refractories. Members of the sillimanite group are valuable for their typical grain structure and expansion upon heating. Of these, kyanite decomposes upon expansion to form mullite at approximately 1200° C. and above, andalusite at 1300° C., and sillimanite at about 1500° C., all of these forming mullite and a fairly refractory glass. Mullite, itself does not expand appreciably on heating, but does not decompose until it reaches 1800° C. and thus is a very efficient refractory.

2263586 01-64x Spodumene, as described in co-pending application, Serial No. 309,784, is the highest expanding material known that possesses a high enough melting point for refractory properties to be useful in the casting of metals, such as alloys of chromium, nickel and cobalt and the like as now used to provide dentures. The use of 1 to 10% of it is generally sufficient to provide adequate expansion and yet promote the use of most any refractory mentioned above.

Other materials that may be used to promote expansion include topaz, pyrophyllite, and baddeleyite, which undergo considerable expansion upon inversion. A number of other silicates undergo slight expansion on inversion. Many new refractories are continuously being made by mixing various proportions of oxides, especially those mentioned above, with each other, and firing them to various temperatures, thus producing refractories that combine the good properties of each.

The refractory aggregate should be properly balanced as to particle size so as to give strength to the investment mold as well as to resist rapid changes in temperature. Strength is achieved by properly grading the refractories as to large, medium, and small particles, each of which fill the interstices between the next larger groups. This maximum density gives strength, but too great a density is not desired, since this causes cracking and also lowers the permeability. Permeability is increased by using a more uniform grading of refractories. Also, the larger the mold size, the larger the coarser material should be. For the usual dental molds, 35 mesh material is generally the coarsest used and with this, 200 mesh material or finer is used. For larger molds, obviously, very coarse refractories, in lump form or crushed rocks, would be desirable in order to preserve the mold shape when heated and prevent cracking and distortion.

From the large number of refractory materials, mentioned as well as similar ones or mixtures thereof (mechanical and chemical), a choice can be made so as to combine practically all desirable features for an investment to be utilized for the casting of metals covering practically the entire fusing range from those melting somewhat above room temperature to those of the highest melting point, such as platinum and its alloys.

When calcium sulphate or plaster is used as the binder, there is a reaction between it and molten metals of fusing points in excess of approximately 2000° F., so that the surface of the casting is rough and there is also porosity due to evolved gases. The evolution of sulphur from the plaster seems to be especially detrimental to alloys containing nickel. When casting metals having a fusing point not much over 2000° F., there is a possibility of producing good castings in plaster molds. It is, however, true that the alloy

composition is extremely limited and in order to overcome this limited condition, a mold should permit casting of metals of higher melting point.

A number of binders are available which do

5 not contain plaster and which generally comprise magnesia and an acid, such as phosphoric acid, has also been practised. The use of sodium silicate promotes vitrification and thus reduces refractoriness and produces a mold that is very difficult to break up and separate from intricate castings. The use of magnesium chloride and magnesia is generally attended with dimensional changes on setting that vary considerably and also this setting expansion may take place some time after the mold has been made. The use of magnesia and phosphoric acid is also subject to an undesirable wide limit of setting expansion. On one occasion it may be very low, approximately .2%, while the same mix under substantially 10 the same conditions may expand up to 1%. This is highly undesirable when extremely accurate work, such as the production of dentures, is to be done and also unusual setting expansions are attended with warpage and cracking of the material.

25 The use of alumina, such as the hydroxide or hydrated oxide along with phosphoric acid generally produces a large shrinkage on setting that is extremely detrimental.

30 The use of metallic zirconates, such as magnesium zirconate and also the respective titanates, as well as double zirconates, such as magnesium zirconium silicate and similar titanates of the metals magnesium, calcium, barium, strontium, zinc, aluminum, sodium, potassium and lithium, along with acids such as phosphoric and other mineral acids is also subject to a wide variety of expansions and contractions on setting. Furthermore, these generally produce an unusual amount of gaseous bubbles in the mix.

35 When adjusted to set fast for general dental use, they also produce an excess amount of heat during the setting, such that the wax pattern is unduly expanded and often distorted, sometimes 40 even melted.

45 It has been found that a very refractory binder and one giving the desired working time and without the undesirable features of unusual variation in the setting expansion, gas evolution, 50 and undue heating will result when magnesia is used in amounts of 3% to 10% along with phosphoric acid of 10% to 40% strength and sufficient amounts of this solution used to form a plastic mass with the refractory and magnesia mixture.

55 To this must be added aluminum in very small amounts, being .02% to .5%, and sometimes up to 1% of the total mixture. This should be preferably dissolved in the liquid, using either the metal, the hydroxide, hydrated oxide, or even the phosphate. These are somewhat less suitable 60 when added to the powder since some of them will not dissolve in time to promote the necessary reaction previous to the final setting of the mix.

65 The amount of aluminum used depends upon the setting expansion desired. The mixture without aluminum when formed into a plastic mass and permitted to set will shrink slightly and then expand rapidly, generally in vary amounts within wide limits. If a very small amount of aluminum, such as .05% be added, the mixture will generally shrink slightly and then expand just enough to make the total setting expansion approximately zero or neutral. Further additions of aluminum will cause the material to shrink somewhat and remain at this figure. Greater additions seem

to promote greater permanent shrankages which are undesirable. The amount of aluminum needed depends upon the type of magnesia used, its grind, and also upon the gradation and size of refractory as well as on the strength of the acid used. These will fall within the comparatively narrow limits set forth above for general use and may be determined by experiment.

If the investment be mixed and used immediately, there will be a slightly lower expansion than if it be mixed and worked until the initial set has set in. By the use of aluminum the variation between the expansions under both conditions are greatly reduced and the material may be used immediately or worked for varying times and still produce accurate results.

When the acid acts on the magnesia, it may form a plastic mass for a while and then set almost instantaneously. This would sometimes spoil the work since the model or upper half of the mix would be only partially poured when the mass set. The use of the small amounts of aluminum seem to promote a more even reaction between the acid and the magnesia.

To promote a still more even reaction and a more regularized setting time, small amounts of magnesium phosphate are desirable and should be used preferably in amounts of .1% to 3% of the mixture. Less than 1% is generally preferable. This may be dissolved in the liquid or added to the powder. The triphosphate is preferable.

The use of this comparatively simple binder with the addition of small amounts of aluminum and magnesia gives a binder that is very refractory. Other metals that form insoluble phosphates may be added either to the liquid or powder, these include principally zinc and cadmium, but their use in appreciable quantities is undesirable since they seem to reduce the refractoriness of the mix. High amounts of aluminum act similarly.

The addition of small amounts of single or double zirconates and titanates when ground to be substantially all through 400 mesh are sometimes of benefit in promoting greater plasticity to the mix and may be used up to approximately 3% of the total composition and generally should be less than half the amount of magnesia used. When magnesium zirconium silicate is used in amounts of 2% or 3%, the use of the small amounts of aluminum in the liquid preferably is more highly desirable to prevent variable setting expansion. The use of these zirconates and titanates also reduces the refractoriness somewhat and causes greater shrinkage of the mold often at high temperatures.

The magnesia may be used in its various forms, that is, in the precipitated form, ignited or fused. The latter is most desirable since it has already been shrunk to its densest state. The magnesia should be used in an amount in excess of that required to react with all of the phosphoric acid. Therefore, there will be an excess of unreacted magnesia present and when not in its densest form will promote shrinkage of the mold. The magnesia should be 200 mesh or finer. The finer the grind, the quicker the reaction and set. For most desirable working qualities, strength, etc., the magnesia should be in quantities more than 5% and the phosphoric acid should be of about 25% or 30% strength. The aluminum should be around 1% and magnesium phosphate .5%.

Ground quartz is the most desirable refractory for dental use but the mold refractory is im-

proved by the use of most refractory materials, such as alumina, silicon carbides, zircon, and the sillimanite group.

The setting time may be controlled by properly balancing the particle size and concentration of the reacting materials, magnesia and phosphoric acid. Heat promotes more rapid reaction, while cooling retards the setting.

Instead of using a mixture of refractory fillers, magnesia, and a liquid consisting of the acid and small amounts of alumina dissolved therein, a double mix of powder may be used. The latter would consist of one powder containing the inert refractory materials and the acid solution, the other powder would consist of the magnesia and magnesium phosphate. The two powders could then be proportioned and the mixture made plastic with water. Likewise, it is possible to add aluminum salts other than the hydroxide or phosphate in order to have the aluminum present to reduce the setting expansion. It is preferable, however, to use an aluminum compound which will form the phosphate when added to the phosphoric acid and without liberating other compounds, such as the chloride, for example, would do.

The proportion of magnesia used and the strength of the phosphoric acid solution control the setting expansion to a considerable extent but when the higher percentages of both are used, the expansion begins to get out of control as explained above and here the aluminum compound controls it as desired. When the magnesia is in the middle of the limits used, the phosphoric acid should preferably be between 25% and 30% strength. The addition of some aluminum compounds, such as the hydroxide, into the phosphoric acid solutions decrease the free phosphoric acid content which also tends to decrease the setting expansion somewhat. With the same strength of free phosphoric acid, the addition of aluminum still gives the desirable advantages of permitting the control of the setting expansion without affecting the percentages of other ingredients which otherwise give a good investment composition.

The use of organic acids and temporary binders, such as gelatin, is not recommended but may be used where certain effects, such as slower setting time, is desired.

The compositions were described above from the standpoint of heating them to red heat and casting at elevated temperatures. Since the setting expansion can be controlled with great accuracy, the molds may be used to reproduce objects accurately at room temperature and even castings could be made therein.

Due also to the neutral setting expansion, it is possible to use the compositions described herein for repairing refractories. The low setting expansion, combined with the other properties of these compositions, permits their adhering to other materials and, since there is no expansion, there is no chance for distortion or cracking. Likewise, these compositions could be used to make objects, such as crucibles, in which metals could be melted.

The above are typical examples of the uses of an investment composition utilizing the magnesia-phosphoric acid-aluminum binder given herein and it is, of course, possible where greater strength is necessary to increase the binder in excess of the amount above set forth so long as the proportions of each ingredient is maintained. Likewise, the compositions given herein could be

used for other purposes than those above set forth in which the properties are desirable.

The above are examples of the manner in which the magnesia-phosphoric acid-aluminum binder may be added to investments and should, therefore, be so considered and not as a limiting factor in the invention.

What is claimed is:

1. An investment composition suitable for making molds into which high melting point metals and alloys may be cast and consisting of a refractory filler making up approximately 85% to 97% of the investment, and the balance being a binder consisting of 3% to 10% of magnesia, and to which is added an aluminum compound capable of forming the phosphate when mixed with phosphoric acid and being present in such amount as to contain .02% to 1% of aluminum, this investment being made into a plastic mass with a solution of phosphoric acid of 10% to 40% strength.

2. An investment composition suitable for making molds into which high melting point metals and alloys may be cast and consisting of a refractory filler making up approximately 85% to 97% of the investment, and the balance being a binder consisting of 3% to 10% of magnesia, this mixture being gaged into a plastic mass with a solution of phosphoric acid of 10% to 40% strength, and containing dissolved therein .02% to 1% of aluminum, based on the weight of the solid ingredients used.

3. An investment composition suitable for making molds into which high melting point metals and alloys may be cast and consisting of a refractory filler making up approximately 85% to 97% of the investment, and the balance being a binder consisting of 3% to 10% of magnesia, this mixture being gaged into a plastic mass with a solution of phosphoric acid of 10% to 40% strength, and containing dissolved therein sufficient aluminum to keep the setting expansion of the investment between .0% and .1% but said aluminum being present not in excess of 1% of the weight of solid ingredients used.

4. An investment composition suitable for making molds into which high melting point metals and alloys may be cast and consisting of a refractory filler making up approximately 85% to 97% of the investment, and the balance being a binder consisting of 3% to 10% of magnesia, and to which is added an aluminum compound capable of forming the phosphate when mixed with phosphoric acid and being present in such amount as to contain .02% to 1% of aluminum, also .1% to 3% of tribasic magnesium phosphate, this investment being made into a plastic mass with a solution of phosphoric acid of 10% to 40% strength.

5. An investment composition suitable for making molds into which high melting point metals and alloys may be cast and consisting of a refractory filler making up approximately 85% to 97% of the investment, of which refractory filler at least 5% is kyanite, and the balance of the composition being a binder consisting of 3% to 10% of magnesia, and to which is added an aluminum compound capable of forming the phosphate when mixed with phosphoric acid and being present in such amount as to contain .02% to 1% of aluminum, this investment being made into a plastic mass with a solution of phosphoric acid of 10% to 40% strength.

6. An investment composition suitable for

making molds into which high melting point metals and alloys may be cast and consisting of a refractory filler making up approximately 85% to 97% of the investment, of which refractory filler at least 5% is kyanite, and the balance of the composition being a binder consisting of 3% to 10% of magnesia, and to which is added an aluminum compound capable of forming the phosphate when mixed with phosphoric acid and being present in such amount as to contain .02% to 1% of aluminum, also .1% to 3% of tri-basic magnesium phosphate, this investment being made into a plastic mass with a solution of phosphoric acid of 10% to 40% strength.

10 7. An investment composition suitable for making molds into which high melting point metals and alloys may be cast and consisting of a refractory filler making up approximately 85% to 97% of the investment, of which refractory filler at least 8% is zircon, and the balance of the composition being a binder consisting of 3% to 10% of magnesia, and to which is added an aluminum compound capable of forming the phosphate when mixed with phosphoric acid and being present in such amount as to contain .02% to 1% of aluminum, this investment being made into a plastic mass with a solution of phosphoric acid of 10% to 40% strength.

20 8. An investment composition suitable for making molds into which high melting point metals and alloys may be cast and consisting of a refractory filler making up approximately 85% to 97% of the investment, of which refractory filler at least 8% is zircon, and the balance of the composition being a binder consisting of 3% to 10% of magnesia, and to which is added an aluminum compound capable of forming the phosphate when mixed with phosphoric acid and being present in such amount as to contain .02% to 1% of aluminum, this investment being made into a plastic mass with a solution of phosphoric acid of 10% to 40% strength.

25 9. An investment composition suitable for making molds into which high melting point metals and alloys may be cast and consisting of a refractory filler making up approximately 85% to 97% of the investment, of which refractory filler at least 8% is zircon, and the balance of the composition being a binder consisting of 3% to 10% of magnesia, and to which is added an aluminum compound capable of forming the phosphate when mixed with phosphoric acid and being present in such amount as to contain .02% to 1% of aluminum, also .1% to 3% of tri-basic magnesium phosphate, this investment being made into a plastic mass with a solution of phosphoric acid of 10% to 40% strength.

40 10. An investment composition suitable for making molds into which high melting point metals and alloys may be cast and consisting of a refractory filler making up approximately 85% to 97% of the investment, of which refractory filler at least 50% is silica, and the balance of the composition being a binder consisting of 3% to 10% of magnesia, and to which is added an aluminum compound capable of forming the phosphate when mixed with phosphoric acid and being present in such amount as to contain .02% to 1% of aluminum, this investment being made into a plastic mass with a solution of phosphoric acid of 10% to 40% strength.

45 11. An investment composition suitable for making molds into which high melting point metals and alloys may be cast and consisting of a refractory filler making up approximately 85% to 97% of the investment, of which refractory filler at least 50% is silica, and the balance of the composition being a binder consisting of 3% to 10% of magnesia, and to which is added an aluminum compound capable of forming the phosphate when mixed with phosphoric acid and being present in such amount as to contain .02% to 1% of aluminum, also .1% to 3% of tri-basic magnesium phosphate, this investment being made into a plastic mass with a solution of phosphoric acid of 10% to 40% strength.

ROBERT NEIMAN.